

Feb. 9, 1932.

S. P. MILLER

1,844,897

PRODUCTION OF LOW CARBON PITCHES

Filed Dec. 29, 1927

2 Sheets-Sheet 1



INVENTOR  
Stuart Parmelee Miller  
BY  
Pennie, Davis, Morris & Edmunds  
ATTORNEYS

Feb. 9, 1932.

S. P. MILLER

1,844,897

PRODUCTION OF LOW CARBON PITCHES

Filed Dec. 29, 1927 2 Sheets-Sheet 2



## UNITED STATES PATENT OFFICE

STUART PARMELEE MILLER, OF ENGLEWOOD, NEW JERSEY, ASSIGNOR TO THE BARRETT COMPANY, OF NEW YORK, N. Y., A CORPORATION OF NEW JERSEY

## PRODUCTION OF LOW CARBON PITCHES

Application filed December 29, 1927. Serial No. 243,305.

This invention relates to the production, at coke oven and other coal distillation plants, of low carbon pitches having predetermined characteristics.

5 In the ordinary operation of by-product coke ovens the gases produced by the coking operation pass from the individual ovens through uptake pipes and goose-necks to a collector main common to the ovens of the battery. The gases which leave the ovens at high temperature, e. g., 600° to 700° C. or higher, are cooled ordinarily as rapidly as possible by the application of sprays of ammonia liquor or ammonia liquor and tar in 10 the goose-necks and collector main. The rapid cooling causes the separation of part of the tar in the collector main. Further cooling is effected in the cross-over main which connects the collector main to the condensing system and in condensing systems and an additional quantity of tar is thus separated. The collected tar is ordinarily mixed and shipped from the coke oven plant to a tar distillation plant for distillation for the 15 separation of the oils and production of pitches.

The pitches produced by distillation of coke oven tar in ordinary tar stills contain too great a proportion of free carbon to make them available for certain uses for which pitches having a low free carbon content are required. For uses such as the saturation of fibre conduits for telephone cables which require a pitch having a low free carbon content, it is customary to employ tar from sources other than coke oven plants. The quantity of material of satisfactory quality available for such uses is, however, relatively limited.

40 It is an object of the present invention to provide a method whereby pitches having a low free carbon content, making them suitable for various purposes for which coal tar pitches are not ordinarily available, may be produced directly at coke oven plants.

It is another object of the invention to produce low carbon pitches at other coal distillation plants or from the tar produced at such plants, such as gas retort plants.

45 During the operation of a coke oven or gas

retort the gases discharged contain a greater or less proportion of tar constituents depending upon the stage of the coking or gas making operation. During the earlier part of the operation the gases discharged from the ovens or retorts contain a relatively large proportion of tar constituents of low carbon content, and the gases, after the separation of the tar, are "rich" gases, rich in illuminants and of high B. t. u. value. Tar separated from such gases is relatively low in free carbon. During the latter part of the coking operation, however, the tar yield decreases and the tar recovered is relatively higher in free carbon content.

According to the present invention, the gases given off from the coke oven or gas retort during an early stage of the coking or gas making operation are separately collected and cooled to separate therefrom a low carbon tar, and this tar is then subjected to distillation to produce therefrom a low carbon pitch of regulated melting point, depending upon the extent to which the distillation is carried. The resulting low carbon pitches will have new and distinctive properties, being distinguished from pitches of the same melting point produced from the total tar from the same ovens by their lower carbon content, lower specific gravity and lower viscosity and different composition, etc. In referring to carbon or free carbon in the tar and pitch I use these terms in the customary way to include not only molecular carbon, but also those materials which appear as an insoluble residue on digestion of the tar or pitch with benzol or other similar solvent. It may include certain inorganic impurities as well as insoluble hydrocarbons of very high molecular weight.

45 In carrying out the invention, advantage is taken of the distinctive characteristics of the tar contained in the gases escaping from the ovens or retorts during different periods of the coking or gas making operation by providing a separate collector main which may be connected to part or all of the ovens or retorts of the battery and by diverting the gases from the ovens or retorts during the required early period of operation into such

55

60

65

70

75

80

85

90

95

100

separate collector main and cooling the gases therein and in separate coolers, to separate therefrom a low carbon tar; and by then keeping this low carbon tar separate and subjecting it separately to distillation for the production therefrom of a low carbon pitch. The gases given off during the remaining period of operation of the coke ovens or gas retorts are separately collected and may be separately cooled to separate therefrom a tar of higher carbon content.

In my companion application, Serial No. 243,307 I have described and claimed a process of producing high carbon pitches by separately collecting the gases from near the end of the coking or gas making operation, cooling these gases to separate a high carbon tar therefrom and distilling the high carbon tar by means of hot coal distillation gases to give a high carbon pitch. The process of said companion application can be carried out at the same plant as the process of the present invention. By combining all of the gases from an arbitrary early period of the coking operation, and by combining the gases from the remaining portion of the coking operation, and separately cooling these gases and separately recovering lower and higher carbon tars therefrom and subjecting these tars separately to distillation, pitches of lower and higher carbon content can be simultaneously produced.

The present invention relates particularly to the production of low carbon pitches by selecting a regulated portion of the gases from the early part of the coking or gas making operation of the individual ovens and separating a low carbon tar therefrom, and subjecting such tar to distillation, whether or not the tar collected from the remaining gases is subjected to distillation or employed for other purposes. If the remainder of the tar is subjected to distillation, the carbon content of the pitch produced will depend upon the particular portion of the coking operation during which the gases are so collected. It is not possible, when dealing with all the gases, with such an arbitrary collection of the gases, to produce a low carbon pitch of regulated carbon content and also produce simultaneously a regulated high carbon pitch other than that normal to the residual gases. Such regulated pitches can, however, be independently and simultaneously produced by providing for the separate collection of the gases during the early, intermediate and later stages of the coking operation and by subjecting the tar separated from such gases to distillation, as set forth in another companion application Serial No. 243,309.

On many coke ovens and in other coal distillation plants equipped with double main gas collecting systems it is possible to collect substantial quantities of several types of high and low carbon tars. For example, in a coke

oven plant of the Semet Solvay type it is customary to limit the number of ovens discharging gas to about twenty per collector main. Thus a sixty oven plant would have three double collector mains, three for rich and three for lean gas. Normally there would be two sets of condensers, one for rich and one for lean gas. The ratio of rich to lean gas may be different in each of the three sets of mains. The greater proportion of the tar in the gases will be thrown out in the collector main and together with the accompanying ammonia liquor can be withdrawn and separated. The individual tars from the three rich and three lean gas mains can thus be regulated in quality. The total rich gases from the three rich gas mains may blend and go to the coolers from which a fourth composite rich gas tar differing from the other three will be collected. Likewise, the lean gases will blend and yield a fourth lean gas tar. While the maximum possible yield of rich gas tar of specific quality can not be obtained by this system as heavy tar from the collector mains, well over 50% of it can be. Such a method of operation has the advantage that it requires no substantial changes in existing equipment, it being necessary only to provide separate pipes for withdrawal of the tars and liquors from the collector mains and coolers and separate tanks for separation of tar and liquors and for storage.

In the operation of the coke oven by-product recovery system for the production of a low carbon tar of regulated low carbon content, I make use of a separate collector main for collecting the gases from part or all of the ovens during a regulated initial period of the coking operation. Two-main systems such as have been employed for the separate collection of "rich" and "lean" gases can be employed, but with regulation of the operation from the stand-point of the carbon content of the tar separated from the gases rather than from the stand-point of the richness or leanness of the gases, after the separation of the tar therefrom. The collector main may be cooled by ammonia liquor sprays, or by the introduction of ammonia liquor and tar therein and the circulation of the liquor and tar therethrough. A considerable portion, usually the greater portion, of the tar can be thus separated as a heavy tar in the collector mains. The tar from the initial period of operation is kept separate from the tar from the later period of operation. That is, the separate collector mains have separate draw-off means for the tar, and the low carbon tar is kept separate. In systems in which the tar is circulated through the collector mains, the tar separated from the gases in each collector main is returned and circulated through the same collector mains so as to avoid admixture of the

low carbon tar with the higher carbon tar produced in the other collector mains.

In addition to collecting separately the low carbon tar from the collector main, a further quantity of low carbon tar is recovered in the condensing system from the same gases. The tar so recovered will ordinarily be a lighter tar or tarry oil. It can be admixed with the heavy tar from the collector main to give a composite low carbon tar, and the composite tar then subjected to distillation for the production of distillate oils and a low carbon pitch; but there are advantages in keeping the heavy tar from the collector main and the lighter tar or tarry oil from the condensers separate from each other and subjecting them separately to distillation. In fractional condensers, a plurality of separate products may be produced, and in some systems a separate product can be drawn off from the end of the cross-over mains just ahead of the condensers. Where a plurality of products are thus fractionally condensed from the gases to produce a series of low carbon tars varying from each other, these can advantageously be distilled separately for the production of the low carbon pitches and of distillate oils.

The distillation of the low carbon tar for the production therefrom of low carbon pitch can be carried out in stills of different types. If the low carbon tar is subjected to distillation in ordinary externally heated stills in which successive charges of tar are distilled to produce successive batches of pitch, considerable decomposition of the tar will take place during the distillation and the carbon content of the resulting pitch will be due in part to the carbon content of the tar distilled and in part to the added carbon formed during distillation. Such pitches will nevertheless be materially lower in carbon than ordinary pitches produced in the same stills from total tar.

A particularly advantageous method of distillation of the low carbon tar for the production of low carbon pitch, is by means of the hot coke oven gases. By bringing the low carbon tar into direct and intimate contact with hot coke oven gases at a high temperature, the tar can be rapidly distilled with a minimum of decomposition and with but small increase in the carbon content of the pitch due to the distillation. Low carbon pitches can accordingly be produced which have a carbon content corresponding to that of the tar from which the pitch is produced, with only a small additional increase resulting from the distillation. Such distillation can be effected, for example, in a separate short distillation main or collector main in which the gases from selected ovens are collected and employed at a high temperature for the distillation, and in which the tar is intimately atomized or sprayed into the gases

to effect the distillation. Gases from the early period of operation of the ovens is advantageously employed for this purpose by distilling the low carbon tar in gases of the kind which contain low carbon tar, the additional tar separated from the gases during the distillation will similarly be of low carbon content. In other cases, the gases from several ovens can be combined during the entire period of operation and employed for the distillation, with some slight increase in carbon content of the resulting pitch due to the somewhat higher carbon content of the tar separated from the gases employed for the distillation. By employing the gases at a high temperature for distillation, the amount of tar distilled will be several times the amount of tar contained in the gases so that the pitch separated from the gases during the distillation will form only a small part of the total pitch product produced by the distillation.

The oils distilled from the low carbon tar are oils of relatively low specific gravity and can advantageously be kept separate from the oils distilled from the remainder of the tar, thus giving an oil of relatively low gravity as one of the products of the process, in addition to the low carbon pitch.

The rate and extent of the distillation can be varied by varying the amount and temperature of the gases employed for the distillation or the rate at which the tar is supplied and the pitch withdrawn. To avoid overheating of the tar and pitch and increase in carbon content as much as possible, the period during which the tar is subjected to heating should be limited. By having only a small body of tar in the still and rapidly atomizing it into the gases and supplying additional tar and drawing off the pitch at a regulated rate, it is possible to carry out the distillation continuously and without prolonged heating of the tar or pitch and with a minimum of increase of carbon content in the pitch produced over that contained in the tar distilled.

In the short collector main or distillation main, the tar and pitch can be atomized or sprayed into the gases by means of spray nozzles or by means of mechanical devices such as discs or cylinders, etc., rotating at high speed and dipping into the body of tar or pitch in the bottom of the short main. Other suitable agitating devices may be employed, the object being to agitate and distribute the tar in the form of relatively small particles throughout the hot gases which flow through the main and to throw the tar upon the exposed surfaces of the main to prevent accumulation of solid pitch thereon.

The distillation of the tar removes a portion of the volatile oil constituents therefrom, leaving a pitch residue which, depending upon the amount of distillation effected, may

have varying characteristics. The distillation results also in the enrichment of the hot gases employed therefor in the volatile oil constituents and such gases may be subjected 5 thereafter to cooling or other treatment to separate the oil constituents therefrom.

The distillate oils produced by the distillation will be relatively clean oils, inasmuch as the distillation will result in enrichment 10 of the gases in oil vapors and the removal therefrom of a considerable part of the suspended pitch particles. Accordingly, relatively clean oils of low specific gravity can be directly produced by cooling the gases employed 15 for the distillation. When the tarry oils from the condensers are kept separate and subjected to distillation separately, the distillate oils will be lighter, or will contain increased amounts of lighter oils. When the heavy tar from the collector main is distilled 20 separately, the yield of oils will be relatively less, but the low carbon pitch will be produced with much less distillation. Accordingly, the heavy tar from the collector main 25 can advantageously be distilled separately to give a relatively high yield of the low carbon pitch with a minimum of distillation, and the tarry oils from the condensers may be employed 30 for other purposes or may advantageously be distilled separately to give a high percentage yield of oils. Where separate low carbon tar fractions are collected in the collector main, at the end of the cross-over main, and at two or more stages of the condensers, 35 all of these four or more fractionally condensed products can be separately subjected to distillation, or only certain of them subjected to distillation, to give a range of distillate oils and low carbon pitches.

As an example of the application of the invention, it may be desirable to produce a low free carbon pitch having a melting point of from 160 to 180° F. (by the air-bath-melting-point method). Such a pitch is suitable for 40 saturating fibre conduits for telephone cables. Pitch of this character can be produced separately, collecting the gases as they are discharged from the coke ovens during the earlier part of the coking operation and by cooling 45 such gases to separate the tar constituents which are distilled thereafter by contact with hot coke oven gases which are given off during the early part of the coking operation. If the proportion of free carbon in the pitch 50 thus recovered is too low for the particular requirements it can be somewhat increased by utilizing ordinary coke oven gases as the distilling media or by adding the required amount of higher carbon tar to the low carbon tar before distillation.

It will be understood that in the practice of the invention the cooling of the "rich" and "lean" gases in the separate collector mains may be regulated by supplying more or less 55 ammonia liquor or other cooling agent there-

to for the purpose of separating a heavier or lighter tar and that by regulation of the amount of oil constituents which are condensed with the tar in the collector mains and by variation of the amount of distillation 70 to which the tar is subsequently subjected, the characteristics of the pitches obtained can be somewhat varied. It will be understood that the recovery of pitches having both low and high free carbon content can be conducted simultaneously in the operation of the same battery and that pitches thus produced can be utilized for any purpose for which they are adapted.

While I have referred more particularly to 80 coke oven operation, and the production of special low carbon pitches from coke oven tar, the invention in its broader aspects includes the production of low carbon pitches in a similar manner at other coal distillation 85 plants and from gas retort tars, etc. Pitches of special properties are obtainable, for example, by separately collecting the tar from the gases given off during the early part of the gas making operation in horizontal inclined or intermittent vertical retorts, and separately distilling such tars. The pitch from the horizontal retort tar will be lower 90 in carbon content, than ordinary pitches from the total tar, and will more nearly resemble pitches from coke oven tar, or blended pitches from mixed coke oven and gas retort tar. The pitches from the low carbon tars at intermittent vertical retort plants will be unusually low in carbon content. The distillates from the distillation of the respective tars will likewise be distinctive.

The present invention is of more or less 100 general application to the operation of coke oven and other coal distillation plants and to the recovery of pitches and oils from the tars separated from the gases discharged therefrom. It will be further described with reference to the accompanying drawings 105 which show apparatus adapted for the practice of the invention, but it is intended and will be understood that the invention is not limited thereto.

Fig. 1 is a plan view of a portion of a coke oven battery illustrating the application of 110 the invention thereto;

Fig. 2 is an enlarged sectional view of one of the collector mains; and

Figs. 3 and 4 are similar views of the short 115 collector main or still in which the tar is distilled.

Referring to the drawings, 5 indicates the battery of ovens which are connected by uptake pipes and goose-necks 6 and 7 to collector mains 8 and 9. Valve boxes 10 and valves 120 11 therein are disposed in the goose-necks to permit the direction of the hot gases from the ovens into one or the other of the collector mains as may be desired. Thus, by operating the valves "rich" and "lean" gases 125

from the several ovens of the battery can be collected separately in the collector mains wherein they are cooled to the desired extent by ammonia liquor, for example, introduced through spray nozzles which are supplied through a pump 13 and pipe 14 from a source of the cooling liquid such as a tank 15.

From the collector mains the gases carrying oil vapors and some tarry constituents are delivered through cross-over mains 16 and 17 to condensers 18 and 19 wherein the gases are subjected to cooling to separate tarry oils therefrom. The tarry oils may be withdrawn through pipes 20 and 21 and delivered to decanters 22 and 23 wherein ammonia liquor is separated from the oils. The tarry oils and ammonia liquor may be delivered to suitable receptacles for storage and subsequent use. The gases may be delivered through pipes 24 and 25 to exhausters 26 and 26' which maintain the pressure balance in the systems and may pass thence to suitable equipment (not shown) for the recovery of ammonia, light oils, etc.

The tar and ammonia liquor from the separate collector mains 8 and 9 may be withdrawn through pipes 45 and 27 and delivered to decanters 28 and 29 in which the ammonia liquor is separated from the tar. The ammonia liquor may be returned for further use as a cooling medium or treated in any suitable manner for the recovery of ammonia therefrom. The tar may be delivered through pipes 30 and 31 to storage receptacles 32 and 33 from which it may be withdrawn as required for further treatment such as distillation to produce pitches.

The distillation of the tar is effected preferably in a suitable still such as a short collector main or still 34 which may be disposed at the rear of the coke oven battery and is connected to a suitable number of ovens through uptake pipes and goose-necks 35 which deliver the hot gases to the short collector main. The tar to be distilled, for example, tar derived from "rich" gases and therefore low in free carbon is delivered by a pump 36 through a pipe 37 to one end of the short collector main or tar box 34 which is provided with a cylinder 38 adapted to be rotated at a high rate of speed by the electric motor 36'. The roll dips into the body of tar and pitch in the bottom of the main or still 34 and by means of the rapid rotation the tar and pitch are atomized, in the form of a finely disseminated spray, into the gases passing through the collector main or still 34. By means of the intimate contact of the tar and gases the former is distilled and pitch is produced which is drawn off at the opposite end of the main or still thru a pipe or thru an outlet 37' and gutter 38' such as shown in Figure 4.

In general the softer pitches will be with-

drawn thru pipes and the harder pitches such as those of 300 to 400° F. melting point and upwards will be withdrawn thru outlets like 37' and gutter like 38'. In case the gutter 38' is used the pitch may conveniently be granulated by allowing it to drop into a stream of water from line 47. The water and granulated pitch will be delivered by the gutter to settling basins 39 from which the pitch may be recovered. In case softer pitches are being made the open gutter is objectionable since it allows excessive fuming of the hot liquid pitch. For that reason a closed pipe line is more desirable.

The hot gases which are partially cooled by contact with the tar and pitch in the short collector main or still are enriched in oil constituents by the distillation effected therein and such gases pass up through settling tower 46 during which passage tar spray and globules and other entrained matter settles out of the gas and is returned to the main or still 34. Tower 46 may be equipped with baffles, packing etc. if desired. The gases can be withdrawn through a pipe 40 and delivered to a condenser 41 located at any suitable place wherein the gases are cooled for the purpose of separating the oil constituents. The oil thus separated can be withdrawn from the condensers through a pipe 42 and delivered to a decanter 43 in which it is separated from ammonia liquor. The oil can be stored in a suitable receptacle and utilized for any desired purpose. The gases, after separation of the oil therefrom, can be delivered by a pipe 44 to the exhauster 26 and mingled with the other gases from the battery, being subjected therewith to the usual treatment for the recovery of ammonia, light oils, etc., therefrom.

The present invention permits the recovery particularly of low free carbon pitches directly from coke oven gases. High free carbon pitches can also be recovered in the same operation together with oils which may be utilized directly or subjected to distillation to separate the oils into various fractions which are adapted for commercial utilization. The invention involves the use of heat available in the coke oven gases to distill the tar recovered therefrom and to produce pitches having the desired characteristics. These and other advantages of the invention may be attained by the practice of the principles as hereinbefore set forth, it being understood that various changes may be made in the details of the operation without departing from the invention or sacrificing the advantages enumerated.

While I have described the invention more particularly in connection with the production of low carbon pitches from coke oven tars, it will be understood that low carbon pitches can similarly be produced at gas retort plants in a similar manner, and that the

different pitches will differ from each other, thus making possible the production of different kinds of pitches at different plants.

I claim:

- 6 1. The method of producing pitch containing a low proportion of free carbon which comprises withdrawing the gases produced during the early stages of coal distillation from a series of ovens or retorts, keeping such
- 10 gases separate from the gases given off during the later stages of distillation, cooling such gases to separate a low free carbon tar therefrom, keeping such tar separate from the tar produced from the gases from the
- 15 later stages of coal distillation, and separately distilling such low free carbon tar to produce pitch of low free carbon content therefrom.
2. The method of producing low gravity
- 20 oils from coal distillation gases, which comprises separately withdrawing the gases produced during the early stages of coal distillation in the ovens or retorts, cooling the gases to separate a heavy tar therefrom, subsequently further cooling the gases to separate a lighter tar therefrom, separately collecting the heavy tar and the lighter tar and separately subjecting the lighter tar to distillation to produce low gravity oils therefrom
- 25
- 30 by bringing such lighter tar into direct and intimate contact with hot coal distillation gases at a sufficiently high temperature to effect rapid distillation thereof.

In testimony whereof I affix my signature.

35 STUART PARMELEE MILLER.

40

45

50

55

60

65